

July 31, 1928.

1,678,826

S. RUBEN

ELECTRIC CURRENT RECTIFIER

Filed April 26, 1927

FIG. 1.



FIG. 2.



FIG. 3.



INVENTOR.  
Samuel Ruben  
BY  
Mayer, Warfield & Nation  
ATTORNEYS.

Patented July 31, 1928.

1,678,826

# UNITED STATES PATENT OFFICE.

SAMUEL RUBEN, OF NEW YORK, N. Y., ASSIGNOR TO RUBEN RECTIFIER CORPORATION, OF ENGLEWOOD, NEW JERSEY, A CORPORATION OF DELAWARE.

## ELECTRIC-CURRENT RECTIFIER.

Application filed April 26, 1927. Serial No. 186,608.

This invention relates to electric current rectifiers and the like, which employ asymmetric couples of the dry surface-contact variety. Rectifiers of this variety are known, which are characterized by the use of a body of relatively electropositive material, employed as one electrode element, disposed in electrical contact with a body of relatively electro-negative material employed as the other electrode element; there being an intervening film having inverse current-blocking properties. Such rectifiers depend for their operation upon the resistance and current-blocking characteristics of the film, which forms as the result of electrochemical action. Rectifiers depending on these characteristics known to the prior art, have been low in efficiency and limited in their application to small current, because of improper conditions for film formation and maintenance, and become substantially inoperative after short periods of use.

This invention has for its object generally to provide an improved device of the character specified, which is efficient, economical and readily manufactured.

More specifically an object of the invention is to provide an asymmetric couple in which the electronegative electrode element is so formed that there is substantially a minimum tendency to the formation of resistance material as a reaction product at the contacting surfaces when passing current, and so arranged that the electrode elements will adjust themselves under varying operating conditions to have substantially maximum contacting area.

Other objects of the invention will in part be obvious and will in part appear herein-after.

The invention accordingly comprises the features of construction, combinations of elements, and arrangement of parts, which will be exemplified in the constructions hereinafter set forth and the scope of the application of which will be indicated in the claims.

For a fuller understanding of the nature and objects of the invention, reference should be had to the following detailed description taken in connection with the accompanying drawing, in which:

Figure 1 shows diagrammatically a rec-

tifying device constructed in accordance 55 with the invention;

Fig. 2 is a view in cross-section showing the electrode elements here employed in assembled arrangement; and

Fig. 3 is a cross-sectional view, similar 60 to Fig. 2, showing a modified arrangement of electrode elements.

Referring now to the drawing, and particularly to Fig. 2, 10 denotes a cup or receptacle having upturned sides, which is made 65 of suitable conducting material; for example, copper, brass or steel. In this cup is disposed a layer of material 11 here employed as the electropositive electrode element. 70

The electronegative electrode element is shown as a plate member, or disc 12, disposed in the cup in co-operative contact with the material 11. The arrangement of the electrode elements is such as to permit assembly by means of a clamping bolt. To this end cup 10, layer 11 and disc 12 are perforated and have an insulating-tube 13 passing therethrough. In order also that the electrical relation of the electrode elements 80 be not disturbed at their outer edge, an insulating-collar 14 is inserted between the up-standing rim of the cup 10 and the edge of the disc 12. 75

The electrode elements thus assembled in 85 cup 10 comprise an asymmetric couple which affords a convenient unit from which to build up a rectifying device of any desired form; for example, as a four-couple device, as shown in Fig. 1. 90

In the arrangement shown in Fig. 1, the couples are arranged in two groups of two couples each, the groups being inverted with respect to each other and disposed conductively against the central conducting terminal plate 15. The couples in turn are separated by interposed conducting terminal-plates 16, there being conducting terminal-plates 17 at the ends of the assembly which are held together under compression 100 by means of a conducting clamping-bolt 18, which has spring-washers 19 interposed between its heads and the end-plates 17. By this arrangement it is seen that the four couples here employed comprise the arms of a Wheatstone bridge, of which the terminals provided at 15 and 18 comprise one diagonal of the bridge circuit, and are 105

adapted to serve as terminals for the output circuit of the rectifying device, here shown as the conductors 20 and 21, leading to the terminals of a direct-current consuming device, here symbolically indicated by the signs + and -.

The terminal-plates 16 disposed intermediate of the groups, serve as terminals for the other diagonal of the bridge circuit, and 10 are employed for making connections to the alternating-current input circuit, here shown as conductors 22 and 23, leading from the low tension side of a suitable step-down transformer 24, which is here shown as 15 connected to an original source 25 of alternating current; for example, a commercial 60-cycle, 110-volt, A.C.-suply.

By the arrangement shown, when the conductor 22 has a plus polarity, the electronegative electrode element in the cup 10 adjacent the terminal-plate 16, to which the conductor 22 leads, will be positively charged, and a direct current will pass, as a result 20 of rectification to the terminal 18, and 25 thence by way of conductor 21 to the plus terminal of the direct-current consuming device, and from thence by way of conductor 20 to a second electronegative electrode element adjacent the terminal-plate 15 to the 30 conductor 23; and vice versa when the conductor 23 has a plus polarity.

In the modified form shown in Fig. 3, the cup 30 is here made of conducting material; this material may be of any suitable 35 kind, for example, molded bakelite. In this form of the device, the electronegative electrode element 32 is in disc-form and is placed in the bottom of cup 30 and has a layer of powdered electropositive material 40 disposed thereon. An insulating tube 33 passes through the rectifying elements and has disposed about it a conducting element 34, such as a plate of copper, for applying 45 pressure to the powdered material under it. These elements are held in operative assembly by the bolt and nut shown at 35 as passing through the insulating tube 33 and applying pressure, when drawn up, through the spring washer 36 to the disc 34 to the 50 rectifying elements beneath. A conducting terminal for the electronegative electrode element is provided which preferably penetrates the insulating cup. This terminal is 55 here shown as a screw 37 secured in cup 30 and in conducting contact with the electronegative electrode element.

This modified form of the invention operates in the same manner as that first described above; the rectifying couple being 60 connected in a circuit, either as a single cell or as a unit having a plurality of cells, by connecting conductors to the terminal 37 and to the bolt 35. The cup 30, however, is here seen to provide a convenient alternative construction for the cup 10 whereby insulating

material is employed instead of conducting material.

The electropositive electrode element here employed is a layer of metallic material in powder form of substantially any relatively 70 suitable, but highly chemically active, electropositive element, for example, aluminum, boron, calcium, magnesium and zinc, as taught in my co-pending application, Serial No. 69,215, filed November 16, 1925. 75

The electronegative electrode element is a body of material which is a compound with, or derivative from, a highly electronegative chemical element, which is adapted to react electrochemically at the contacting surface 80 with the electropositive material to form an inverse current-blocking film. Metallic compounds with the elements of the sixth group in the periodic table are suitable compounds from which to provide the material 85 for the electronegative electrode element, as also set forth in my co-pending application above referred to. In this prior application it was pointed out as desirable to employ a metallic alloy as the basic metallic material 90 to be compounded with the chemical elements of the sixth group, since a body of material is thereby provided having sufficient resistance to impart inherent film-forming properties to the asymmetric couple. 95

A reaction product is electrochemically formed at the contacting surfaces of the electrode elements, in addition to the inverse current-blocking film which gradually increases in resistance, thereby cutting down the useful life of the couple. The rate of the formation of this reaction product is roughly inversely proportional to the density of the electronegative electrode element. As this element is generally a compound in crystal form, this density is herein referred to as the "crystal density". It has been ascertained that the crystal density and mechanical strength and rigidity of the electronegative electrode element may be increased together by the addition of further alloy material which is metallic in nature, imparting hardness, but does not decrease the electronegative character of the electrode element. The material suitable for this purpose consists of the refractory metals of the sixth periodic group, sometimes referred to as "sub-group B" thereof; namely, the metals chromium, molybdenum and tungsten. Each of these latter metals is obtainable commercially in oxide form, which oxides have been ascertained to be suitable forms to be added to the basic material of the electrode element. These elements may be taken in amounts up to substantially 20% by weight 120 of the total mass of the electronegative electrode when accomplishing the object of the invention. 125

The following is an example of suitable components for the electronegative electrode 130

element, which reacts well with an electropositive electrode element of powdered magnesium:

|                   | Per cent. |
|-------------------|-----------|
| 5 Cupric sulphide | 75        |
| Zinc sulphide     | 10        |
| Selenium          | 5         |
| Chromium trioxide | 10        |

These materials are fused together at a temperature of substantially 1300° C. and are cast into discs or small plates.

In order to insure maximum density, the cast plates, while still plastic, are worked by mechanically rolling the same until reduced from one-half to one-third of their original thickness. This working preferably takes place at a temperature of about 600° C.

When electronegative electrode elements are thus produced, they have substantial maximum density for the material employed, and when assembled in contact with the powdered electropositive electrode element in the cup 10, together they form an asymmetric couple that is highly resistant to the formation of any reaction-resistance product at their contacting surfaces. Such couples, when assembled, as indicated in Fig. 1, have pressure applied to them as set forth in my co-pending application, Serial No. 38,781, filed June 20, 1925, in order to prevent the inverse current-blocking film from being disrupted by the forces of electrostatic repulsion that operate at the contacting surfaces when rectifying current passes. By employing an electropositive electrode element in powder form, it is seen that it is adapted to adjust itself for intimate contact with the surface of the electronegative electrode element so that there is substantially a maximum of conducting area under all conditions of operation, thereby insuring that the device may be operated at substantially maximum current densities without danger of destroying the inverse current-blocking film by overheating at any point in the contacting surface. The couple thus provided consequently has high stability and is adapted to give a relatively long life under relatively severe operating conditions.

Since certain changes may be made in the above construction and different embodiments of the invention could be made without departing from the scope thereof, it is intended that all matter contained in the above description, or shown in the accompanying drawing, shall be interpreted as illustrative and not in a limiting sense.

Having described my invention, what I claim as new and desire to secure by Letters Patent is:

1. In dry surface-contact rectifying devices and the like, an asymmetric couple having an electronegative electrode element comprising a metallic compound of the sixth

periodic group, having substantially maximum crystal density, an electropositive electrode element comprising highly electropositive metallic material in powder form, and means for retaining said electrode elements in contact under pressure sufficient to prevent the disruption of the inverse current-blocking film which forms at the contacting surfaces of said electrodes.

2. In dry surface-contact rectifying devices and the like, an asymmetric couple having an electronegative electrode element comprising a metallic compound of the sixth periodic group, having substantially maximum crystal density, and which is relatively highly resistant to the formation of reaction resistance products, an electropositive electrode element comprising highly electropositive metallic material in powder form, a containing cup adapted to hold said electropositive electrode element in co-operative contact with said electronegative electrode element, and means for retaining said electrode elements in contact under pressure sufficient to prevent the disruption of the inverse current-blocking film which forms at the contacting surfaces of said electrodes.

3. In dry surface-contact rectifying devices and the like, an asymmetric couple having an electronegative electrode element comprising a compound of the sixth periodic group with an alloy, having a relatively highly-conducting metallic component, a second metallic component adapted to increase the resistance thereof and to increase the density, durability and resistance to the formation, electrochemically, of reaction-resistance products on the surface thereof, an electropositive electrode element comprising highly electropositive metallic material in powder form, a containing cup for holding the latter in co-operative contact with the electronegative electrode element, and means for retaining said electrode elements in contact under pressure sufficient to prevent the disruption of the inverse current-blocking film, which forms at the contacting surfaces of said electrodes.

4. In dry surface-contact rectifying devices and the like, an asymmetric couple having an electronegative electrode element comprising a compound of the sixth periodic group with an alloy containing copper and a relatively highly refractory electronegative metallic element, adapted to increase the crystal density of said electrode element and to render the same resistant to the formation of reaction resistance products, an electropositive electrode element comprising highly electropositive metallic material in powder form, a containing cup adapted to contain said electrode elements in contact, means for insulating the edges of said electrode elements within said cup, and means for retaining said electrode elements in contact

under pressure sufficient to prevent the disruption of the inverse current-blocking film which forms at the contacting surfaces of said electrodes.

5. In dry surface-contact rectifying devices and the like, an asymmetric couple having an electronegative electrode element comprising a compound of the sixth periodic group with an alloy containing copper, zinc and chromium, taken in proportions adapted to impart high crystal density and to render the same relatively highly resistant to the electrochemical formation of reaction resistance products on the surface thereof, 10 an electropositive electrode element comprising metallic magnesium in powder form; a containing cup adapted to contain said powder material and to support said electronegative electrode element in contact with 15 the electropositive electrode element, insulating means inserted in said cup and adapted to insulate the edges of said electrode elements, and means for retaining said electrode elements in contact under pressure sufficient to prevent the disruption of the 20 inverse current-blocking film which forms at the contacting surfaces of said electrodes.

6. In dry surface contact rectifying devices and the like, an asymmetric couple having electronegative electrode elements comprising a compound of the sixth periodic group with an alloy containing copper, zinc and chromium taken in proportions adapted to impart high crystal density and to render 25 the same relatively highly resistant to the electrochemical formation of reaction resistance products on the surface thereof, an electropositive electrode element comprising highly electropositive metallic material in 30 powdered form, a containing cup adapted to contain said electrode elements disposed in operative contact, means for insulating the edges of said electrode elements, a closure for said cup, and resilient means bearing 35 on said closure adapted to retain said elec- 40

trode elements in contact under pressure sufficient to prevent the disruption of the inverse current-blocking film which forms at the contacting surfaces of said electrodes.

7. In dry surface contact rectifying devices and the like, an asymmetric couple having electronegative electrode elements comprising a compound of the sixth periodic group, with an alloy containing copper, zinc and chromium taken in proportions adapted to impart high crystal density and to render the same relatively highly resistant to the electrochemical formation of reaction resistance products on the surface thereof, an electropositive electrode element comprising metallic magnesium in powdered form, a containing cup adapted to contain said electrode elements disposed in operative contact, means for insulating the edges of said electrode elements, a closure for said cup, and resilient means bearing on said closure adapted to retain said electrode elements in contact under pressure sufficient to prevent the disruption of the inverse current-blocking film which forms at the contacting surfaces of 50 55 60 65 70 75 80 85 90 95 100 said electrodes.

8. In dry surface contact rectifying devices and the like, an asymmetric couple comprising a pair of electrode elements, one in powdered form, the other in solid form, a containing cup adapted to contain said electrode elements disposed in operative contact, insulating means associated with said cup and adapted to maintain the edges of said elements in proper insulated relation, means consisting of a freely-moving member for closing said cup, and clamping means adapted to bear on said closing means arranged to maintain said electrode elements in contact under pressure sufficient to prevent a disruption of the inverse current-blocking film which forms at the contacting surfaces of said electrodes.

In testimony whereof I affix my signature.  
**SAMUEL RUBEN.**